

## UNITED STATES PATENT OFFICE

2,573,933

## STABILIZATION OF MOTOR FUELS

Louis Schmerling, Riverside, and Joseph A. Chenicek, Bensenville, Ill., assignors to Universal Oil Products Company, Chicago, Ill., a corporation of Delaware

No Drawing. Application February 8, 1949,  
Serial No. 75,307

4 Claims. (Cl. 44—63)

**1**  
This invention relates to the stabilization of motor fuels which tends to deteriorate in storage due to oxidation reactions. It is an object of the present invention to prevent or at least substantially retard the undesirable deterioration of motor fuels comprising olefinic gasolines such as cracked gasoline and polymer gasoline.

In a broad embodiment, the present invention relates to a method of stabilizing motor fuels which comprises incorporating therein an inhibitor comprising a hydroxyphenylpiperidine.

In a specific embodiment, the present invention relates to a method of stabilizing cracked gasoline which comprises incorporating therein from about 0.0001% to about 0.1% by weight of 1-(p-hydroxyphenyl)-4, 4-dimethylpiperidine.

The preferred inhibitor of the present invention comprises hydroxyphenyl-piperidines and particularly 1-(p-hydroxyphenyl)-4, 4-dimethylpiperidine which is illustrated in the following formula.



These compounds may readily be prepared by the reaction of a 1, 5-dihaloalkane with p-aminophenol or by the reaction of hydroquinone with a piperidine. The reaction is readily effected by refluxing the reactants at a suitable temperature which may range from about 50° to about 200° C. and preferably is of the order of 75° to 125° C. A suitable solvent such as dioxane may be utilized in the preparation of the compound, and the dioxane may be distilled off and the residuum extracted with a suitable solvent and recovered by recrystallization.

Referring to the structural formula hereinbefore set forth, it is understood that the aromatic ring and/or the heterocyclic ring may contain various further substituents including alkyl, aryl, aralkyl, alkaryl, alkoxy, aralkoxy, hydroxy, etc., radicals and that these alternative, but not necessarily equivalent, compounds may be prepared by further alkylating the above compound or by the use of other starting materials in the preparation of these inhibitors.

In the preferred inhibitors of the present invention, the hydroxy radicals attached to the aromatic ring is in a position para to the nitrogen atom. However, it is understood that compounds in which the hydroxy group is in the ortho or meta position are comprised within the scope of the present invention and that these various compounds are not necessarily of equivalent activity.

**2**  
The inhibitor of the present invention will usually be added to gasoline in an amount of less than 0.5% by weight and generally will be utilized in an amount of from about 0.0001% to about 0.1%. The exact amount of inhibitor required will depend upon the particular motor fuel being treated and upon the stability desired. These inhibitors may also be employed in connection with various dyes, antiknock agents such as tetraethyl lead, metal deactivators or other additives employed for specific purposes in the motor fuel.

The following example is introduced to illustrate further the novelty and utility of the present invention but not with the intention of unduly limiting the same.

1 - (p-hydroxyphenyl) - 4,4 - dimethylpiperidine was prepared as follows: A solution of 11 g. of p-aminophenol and 13 g. of 1,5-dibromo-3,3-dimethyl pentane in 53 g. of dioxane was refluxed at 103° C. for 12 hours. The dioxane was distilled off and the residue was extracted with ether and recrystallized from alcohol to recover the desired compound having a melting point of 129-130° C.

The above compound was tested as an inhibitor in cracked gasoline which had a blank induction period of 45 minutes. 0.005% of the compound prepared in the above manner was added to the cracked gasoline. The induction period of the cracked gasoline was increased from 45 minutes to 365 minutes upon the addition of the inhibitor. The induction period is determined by the Oxygen Bomb Stability Test which is a standard method for evaluating the storage stability of gasoline.

We claim as our invention:

1. Olefinic gasoline containing a small amount of a 1-hydroxyphenyl-piperidine, sufficient to retard oxidative deterioration of the gasoline.
2. Cracked gasoline containing a small amount of 1-(p-hydroxyphenyl)-4,4-dimethylpiperidine, sufficient to retard oxidative deterioration of the gasoline.
3. Cracked gasoline containing from about 0.0001% to about 0.1% by weight of 1-(p-hydroxyphenyl)-4,4-dimethylpiperidine.
4. Olefinic gasoline containing a small amount of a 1-(p-hydroxyphenyl)-piperidine, sufficient to retard oxidative deterioration of the gasoline.

LOUIS SCHMERLING,  
JOSEPH A. CHENICEK.

## REFERENCES CITED

55 The following references are of record in the file of this patent:

## UNITED STATES PATENTS

Number Name Date  
60 2,300,246 Chenicek et al. Oct. 17, 1942